

## UNITED STATES PATENT OFFICE

2,512,590

## CORROSION INHIBITORS

Robert C. Swain, Riverside, and Joseph H. Paden,  
Glenbrook, Conn., assignors to American Cy-  
anamid Company, New York, N. Y., a corpora-  
tion of Maine

No Drawing. Application March 31, 1942,  
Serial No. 436,976

1 Claim. (Cl. 260—249.5)

1

This invention relates to the prevention of corrosion in processes wherein cyanamide or its dimer, dicyandiamide, is converted to other organic compounds by processes wherein these materials are heated at high temperatures and pressures in the presence of solvents containing ammonia. More particularly, it embraces the production of such products in a condition substantially free from contamination by iron, nickel or similar metallic impurities by carrying out the conversion in stainless steel autoclaves and in the presence of inhibitors such as phosphates, chromates, and the like.

It is well known that cyanamide and dicyandiamide are important raw materials for the production of a great number of organic nitrogen compounds. For example, melamine can readily be prepared by reacting a charge consisting of 1 part of cyanamide or dicyandiamide, 1 to 2 parts of anhydrous ammonia and 1 to 2 parts of methyl alcohol or a similar organic solvent at a temperature of 120°—200° C., over a period of 4 to 12 hours. Various modifications of this process result in the production of guanidine salts, as by introducing equivalent quantities of the corresponding ammonium salts into the reaction mixture.

Heretofore, it has been found that when such reactions are carried out in autoclaves made from alloys such as those known commercially as high-chrome or stainless steels, the products are contaminated with an excessive amount of undesirable impurities since the autoclaves, fabricated from such iron alloys with about 8-20% of chromium content based on the total weight of the alloys, although somewhat resistant to the attack of such mixtures are nevertheless slightly corroded. This results in products containing undesirable quantities of iron, nickel and similar impurities which are derived directly from the alloys used in the autoclaves.

It is an object of the present invention to provide a method for protecting these mixtures and the autoclaves wherein they are reacted from the corrosive effects of the conversion products of cyanamide, dicyandiamide and similar organic compounds. It is a further object of this invention to provide a method for the protection of chrome-alloy or chrome-nickel alloy steel apparatus used in handling and processing cyanamide, dicyandiamide, guanidine nitrate and similar compounds. A further object of the present invention is to improve the above and similar conversion processes by conducting them in iron and chromium alloy autoclaves in the presence of corrosion inhibitors such as diammonium phosphate, ammonium dichromate, sodium dichromate, and the like, in order to obtain products that are substantially free from contamination by iron, nickel, and the like.

Broadly speaking, the invention embraces bathing or wetting, continuously or intermittently, the metallic surfaces exposed to the conversion

2

products of cyanamide, dicyandiamide, guanidine nitrate, and the like, with a liquid containing diammonium phosphate, ammonium dichromate, sodium dichromate, and similar corrosion inhibitors. These inhibitors are preferably present in concentrations of from 50 to 1000 parts per million, based on the total autoclave charge.

It is well known that ordinary ammonia, whether aqueous or anhydrous, is not corrosive to unalloyed iron or steel at temperatures extending up to 400° C. It is also known that neither cyanamide nor dicyandiamide attack iron or steel when these compounds are stored in containers or shipped in such containers. Solutions of cyanamide or dicyandiamide in liquid ammonia, whether treated with methyl, ethyl or similar alcohols, have likewise been found to be non-corrosive. However, when such solutions of cyanamide and dicyandiamide in liquid ammonia are heated to temperatures whereat they are converted to such products as melamine, guanidine nitrate, and the like, it has been found that ordinary steel autoclaves and even autoclaves prepared from stainless steels containing from 8% to 20% of chromium and up to 8% of nickel are rapidly attacked and the product is seriously discolored and contaminated with such impurities as iron, nickel, chromium, and the like.

This rapid attack by cyanamide and dicyandiamide solutions in liquid ammonia during conversion upon the walls of an autoclave assumes very serious proportions, since ferrous equipment is the only commercially available material that will withstand the great pressures involved in this type of conversion. For example, in the process for the manufacture of melamine, autoclave pressures of 3000 pounds per square inch are not uncommon and similar pressures are also necessary for the production of other guanidine salts. If non-ferrous equipment were to be used, an autoclave capable of withstanding such pressures safely would be extremely expensive to design and maintain if commercial batches were to be produced.

In accordance with one embodiment of this invention, it has been found that a class of ferrous alloys known as high-chrome steels, alloys of iron containing about 8-20% of chromium based on the total weight of the alloys and stainless steel, are capable of withstanding the pressures above mentioned with a large factor of safety, and can be used to fabricate autoclaves. When from 50 to 500 or more parts per million of inhibitors such as ammonium phosphate, ammonium dichromate, sodium dichromate, and the like, are added to the reaction mixture in such autoclaves, products containing very little, if any, ferrous and similar impurities are obtained. The above high-chromium steel alloys are usually referred to as low carbon steels, since they contain from about .06% to about .2% of carbon, and in addition varying proportions of other ele-

ments such as smaller percentages of sulfur, selenium, and silicon, and not more than about 15% of nickel. Such alloys as contain nickel are preferably stabilized by the addition of molybdenum, columbium, titanium, manganese, or mixtures of two or more of such elements up to approximately ten times the amount of carbon present. Usually from 8-12% of nickel is present in these alloys. This improves their machining properties and facilitates their fabrication. However, more than 15% of nickel tends to increase corrosion in the alloys.

The conversions of cyanamide or dicyandiamide embraced by this invention are effected in mixtures containing liquid ammonia in the autoclaves above described and preferably at high temperatures and pressures. Usually the autoclaves are fabricated from or lined with the above alloys. The reactions are carried out without corrosion of the alloy liner or autoclave, and without excessive contamination of the product with iron, nickel or other metallic impurities contained in the alloy, by adding effective amounts of the corrosion inhibitors given in more detail hereafter. The addition of such corrosion inhibitors results in a remarkable resistance on the part of the alloy to corrosion during the reaction. The purity of the products obtained is further illustrated by the following examples, which, however, are not intended to limit the invention except as further defined in the claims.

In each of the following examples, an autoclave fabricated from a high-chrome steel or fitted with a liner made of a high-chrome steel was charged with a mixture containing 450 g. of liquid ammonia, 473 g. of ammonium nitrate containing at most 12 parts per million of iron and 250 g. of dicyandiamide containing 5 parts per million of iron. This reaction mixture was heated to 160° C. over a period of about one hour and held at 160° C. for an additional hour whereupon it was cooled and a pure white guanidine nitrate obtained in those cases where an inhibitor was used in effective amounts.

TABLE I

| Example | Inhibitor | Parts per Million |        | Product    |
|---------|-----------|-------------------|--------|------------|
|         |           | Iron              | Nickel |            |
| 1.      | None      | 7,150             | 1,030  | Very dark. |
| 2.      | do.       | 15,100            | 2,130  | Do.        |
| 3.      | do.       | 20,800            | 2,910  | Do.        |
| 4.      | do.       | 8,870             | 1,330  | Do.        |
| 5.      | do.       | 19,540            | 2,800  | Do.        |
| 6.      | do.       | 10,400            | 1,430  | Do.        |
| 7.      | do.       | 12,500            | 1,560  | Do.        |
| 8.      | do.       | 12,900            | 2,140  | Do.        |
| 9.      | do.       | 6,250             | 930    | Do.        |
| 10.     | do.       | 7,930             | 1,120  | Do.        |
| 11.     | do.       | 24,630            | 3,800  | Do.        |

In the first three runs the liner of the autoclave lost 23.5 grams during the experiments.

During the remaining runs the liner lost 94 grams in weight. This clearly indicated that corrosion of the liner contributed to the greater part of the contamination of the product.

5 In order to see whether the use of iron or nickel alloys stabilized with molybdenum or columbium which were given a metallo-graphic finish by pickling them in a nitric acid-hydrofluoric acid bath and subsequently passivating them in a warm 20% nitric acid bath, liners having the composition shown in Table II were used to prepare melamine using the following charge:

10 Equal parts by weight of dicyandiamide, liquid ammonia and commercial methanol were heated in the autoclave reaching a temperature of 180° C. over a period of one hour. The charge was held at 180°-190° C. for two more hours after which it was cooled to room temperature and the contents removed. The products contained on 20 an average of 0.034% of iron.

TABLE II

| Example | Per Cent Composition (balance iron) |      |      |      |      |       |       | Loss of Weight, grams |
|---------|-------------------------------------|------|------|------|------|-------|-------|-----------------------|
|         | C                                   | Cr   | Ni   | Si   | Mn   | Mo    | Co    |                       |
| 12.     | 0.15                                | 18.0 | 10.0 | 0.75 | 0.75 | ----- | 1.2   | 0.0043                |
| 13.     | 0.08                                | 19.0 | 8.0  | 0.75 | 0.75 | ----- | ----- | 0.0114                |
| 14.     | 0.25                                | 25.0 | 20.0 | 2.00 | 1.20 | ----- | ----- | 0.0322                |

30 The material produced in each of the various runs is thus seen to be unduly contaminated with iron, nickel and similar impurities. Because of this, the following runs were made using the 35 inhibitors indicated with the reaction mixture used in the examples of Table I.

TABLE III  
Ammonium dichromate inhibitor

| Example | Parts per Million |      |        |          | Product      |
|---------|-------------------|------|--------|----------|--------------|
|         | Inhibitor         | Iron | Nickel | Chromium |              |
| 15.     | 1,000             | 46   | 4      | 512      | Slight pink. |
| 16.     | 1,000             | 16   | <1     | 550      | Do.          |
| 17.     | 1,000             | 11   | <1     | 950      | Do.          |
| 18.     | 1,000             | 14   | -----  | 275      | White.       |

TABLE IV  
Diammonium phosphate inhibitor

| Example | Parts per Million |      |        |          | Product           |
|---------|-------------------|------|--------|----------|-------------------|
|         | Inhibitor         | Iron | Nickel | Chromium |                   |
| 19.     | 2,000             | 18   | <1     | <1       | Excellent, white. |
| 20.     | 1,500             | 15   | <1     | 1        | Do.               |
| 21.     | 1,000             | 12   | <1     | 1        | Do.               |
| 22.     | 1,000             | 13   | <1     | 1        | Do.               |
| 23.     | 500               | 17   | 1      | 1        | Do.               |

TABLE V  
Diammonium phosphate inhibitor

| Example | Parts per Million       |      |        |          | Product           |
|---------|-------------------------|------|--------|----------|-------------------|
|         | Inhibitor               | Iron | Nickel | Chromium |                   |
| 24.     | 2,000                   | 14   | 2      | 1        | Excellent, white. |
| 25.     | 1,000                   | 14   | <1     | <1       | Do.               |
| 26.     | 500                     | 13   | <1     | <1       | Do.               |
| 27.     | None, liner of 26 used. | 13   | 1      | <1       | Do.               |
| 28.     | Same as 27.             | 16   | 1      | <1       | Do.               |
| 29.     | do.                     | 20   | 1      | 2        | Do.               |

This series of experiments showed that by using an inhibitor, a passivated film is formed on the liner which retains its effectiveness for several runs thereafter.

TABLE VI  
*Diammonium phosphate inhibitor*

| Example | Parts per Million |        |        |          | Product |                   |
|---------|-------------------|--------|--------|----------|---------|-------------------|
|         | Inhibitor         | Iron   | Nickel | Chromium |         |                   |
| 30..... | None              | 11,100 | 1,350  |          | 4,200   | Very dark.        |
| 31..... | 125               | 65     | 2      |          | 4       | Excellent, white. |
| 32..... | 125               | 16     | 4      |          | 2       | Do.               |

In order to determine the minimum amount of inhibitor necessary for effective prevention of corrosion, the following experiments were carried out in accordance with previous autoclave charges.

TABLE VII  
*Diammonium phosphate inhibitor*

| Example | Parts per Million       |        |        |          | Product |                   |
|---------|-------------------------|--------|--------|----------|---------|-------------------|
|         | Inhibitor               | Iron   | Nickel | Chromium |         |                   |
| 33..... | None                    | 13,650 | 1,600  |          | 3,600   | Very dark.        |
| 24..... | 25                      | 12,900 | 1,510  |          | 4,000   | Rather dark.      |
| 35..... | 50                      | 57     | 4      |          | 7       | Excellent, white. |
| 36..... | 50                      | 39     | 2      |          | 4       | Do.               |
| 37..... | 75                      | 23     | 1      |          | 2       | Do.               |
| 38..... | 75                      | 17     | 1      |          | 2       | Do.               |
| 39..... | None, liner of 38 used. | 25     | 2      |          | 3       | Do.               |
| 40..... | Same as 39.....         | 8,370  | 460    |          | 2,600   | Rather dark.      |

From these experiments it is seen that at least 50 or more parts per million of the inhibitor are necessary to prevent contamination of the product. Moreover, with the small amount of inhibitor used, although the liner of Example 39 was still effectively passivated, the next run (Example 40) showed that only a very thin protecting layer was present (compare Table V).

TABLE VIII  
*Ammonium chromate inhibitor*

| Example | Parts per million |       |        |          | Product           |
|---------|-------------------|-------|--------|----------|-------------------|
|         | Inhibitor         | Iron  | Nickel | Chromium |                   |
| 41..... | None              | 9,370 | —      | —        | Dark color.       |
| 42..... | 500               | 40    | —      | —        | Excellent, white. |
| 43..... | 250               | 21    | —      | —        | Do.               |
| 44..... | 100               | 17    | —      | —        | Do.               |

Since iron was the principal contaminating material, these examples were analyzed for the presence of iron only.

TABLE IX  
*Sodium dichromate inhibitor*

| Example | Parts per million |       |        |          | Product           |
|---------|-------------------|-------|--------|----------|-------------------|
|         | Inhibitor         | Iron  | Nickel | Chromium |                   |
| 45..... | None              | 1,890 | 160    | 680      | Slightly colored. |
| 46..... | 500               | 18    | 2      | 1        | Excellent, white. |
| 47..... | 250               | 16    | 1      | —        | Do.               |
| 48..... | 100               | 18    | 2      | 7        | Do.               |
| 49..... | 100               | 21    | 1      | 1        | Do.               |

In a manner similar to those given above for the production of melamine and guanidine nitrate, the same inhibitors, in the same propor-

tions can effectively be used to prevent corrosion of the autoclave and contamination of the product when used to prepare guanidine carbonate from reacting proportions of dicyandiamide, ammonium carbonate and water in the presence of liquid ammonia.

The examples herein given clearly show that ordinary high-chrome steels are not in themselves satisfactory corrosion resistant materials for reactions wherein cyanamide or dicyandiamide is a reagent. Moreover, it is to be understood that various other chromate or chromate-ion-containing compounds such as various other alkali-metal chromates, namely potassium chromate and bichromate among still other chromate metallic salts, can be used and are to be considered as embraced within the broad limits of this invention.

It is to be understood that the examples given

in detail are merely illustrative and not limitative embodiments of the invention, the scope of which is more clearly indicated in the following claim.

40 We claim:  
In the conversion of a compound selected from the group consisting of cyanamide and dicyandiamide to a derivative thereof, and including the step which consists in heating said compound while dispersed in a solvent comprising liquid ammonia in a closed pressure vessel in which all the internal surfaces in contact with the reaction mixture consist of a ferrous alloy selected from the group consisting of high-chrome and stainless steel, the improvement which consists in protecting the metallic surfaces exposed to the reaction mixture by adding from 50 to 1000 parts of ammonium phosphate per million parts of the reactants.

55 ROBERT C. SWAIN.  
JOSEPH H. PADDEN.

#### REFERENCES CITED

60 The following references are of record in the file of this patent:

#### UNITED STATES PATENTS

| Number       | Name         | Date           |
|--------------|--------------|----------------|
| 65 1,841,825 | Kriegsheim   | Jan. 19, 1932  |
| 1,875,982    | Boller       | Sept. 6, 1932  |
| 1,988,584    | Dana         | Jan. 22, 1935  |
| 2,056,283    | Lawrence     | Oct. 6, 1936   |
| 2,129,689    | Hetherington | Sept. 13, 1938 |
| 70 2,191,361 | Widmer       | Feb. 20, 1940  |
| 2,273,781    | Hochwalt     | Feb. 17, 1942  |

#### OTHER REFERENCES

Snell: Industrial and Engineering Chemistry, 75 Vol. 23, No. 5, page 474, May 1931.